

J. G. WEST, JR.  
METHOD OF SINTERING FINE ORES AND SIMILAR MATERIALS.  
APPLICATION FILED JAN. 4, 1912.

1,031,153.

Patented July 2, 1912.



## **WITNESSES**

R.S. Little  
Chas. Fosterman

## INVENTOR

INVENTOR  
J. G. West Jr.  
by Lathicium Beltr. Fuller  
his Attorney

# UNITED STATES PATENT OFFICE.

JAMES G. WEST, JR., OF WILKINSBURG, PENNSYLVANIA.

## METHOD OF SINTERING FINE ORES AND SIMILAR MATERIALS.

1,031,153.

specification of Letters Patent.

Patented July 2, 1912.

Application filed January 4, 1912. Serial No. 689,474.

To all whom it may concern:

Be it known that I, JAMES G. WEST, Jr., a citizen of the United States, residing at Wilkinsburg, in the county of Allegheny 5 and State of Pennsylvania, have invented a new and useful Method of Sintering Fine Ores and Similar Materials, of which the following is a specification.

My invention relates to the agglomeration 10 of finely divided materials such as iron ores, flue-dust, mill scale, slag and similar granular or finely divided solids, in which a quantity of such materials is sintered or burned into an integral mass by the application of 15 heat.

One object of my invention is to provide a novel method of sintering such finely divided solids whereby the particles of the materials are softened by the application of 20 heat and are fused or are partly fused or welded together and caused to adhere and form an integral mass or clinker.

Another object of the invention is to provide an improved method of sintering ores 25 and finely divided materials generally having novel means whereby successively added quantities of the materials are caused to fuse or partly fuse and adhere in forming and building up a substantial mass of such ma- 30 terial.

A further object of this invention is to provide a novel method of sintering such materials by the use of which an integral mass of the materials is gradually built up 35 and is then broken into pieces of suitable size for charging into a blast furnace or other metallurgical furnace.

Referring to the accompanying drawings forming part of this specification, Figure 1 40 is a longitudinal sectional elevation showing a furnace as constructed and arranged for use in carrying out the steps of my improved method. Fig. 2 is a sectional end elevation of the same on the line II—II of 45 Fig. 1.

In the drawings, a reverberatory furnace 2 is shown having a series of burners 3 arranged at intervals along the sides thereof. A series of passages 4 in one side thereof 50 communicate with the stack 5. A vertically extending opening 6 is formed in approximately the lengthwise and transverse center of the roof 7 of the furnace, for a purpose described later.

55 The bottom of the furnace is built up of a suitable refractory material 8 which is

placed upon a body or framework 9 provided for that purpose. The framework 9 is mounted on wheeled trucks 10, the wheels of which travel on the track rails 12 passing lengthwise through the furnace 2 so that the bottom of the furnace is movable into and out of the furnace chamber. A series of these removable bottoms preferably are employed in carrying out my improved method. 60

In carrying out the steps of my improved method, the movable furnace bottom is first prepared by building a wall 13 along the marginal edges of its top surface so as to form a rectangular inclosure. Refractory 70 clays, stone or brick, or other material having heat resisting qualities equal to those of the materials to be treated are employed in building this marginal wall 13 on the furnace bottom 8. A layer of the ore, flue dust, 75 mill scale or other finely divided material is then spread over the furnace bottom within the inclosure formed by the marginal wall 13, the material used preferably being of the same composition as that to be sintered. The 80 layer of finely divided material is made of such thickness that the material will not stick to the refractory bottom, the thickness of this layer being sufficient to prevent its being entirely heated to a plastic state. 85

The furnace bottom, after preparation in this manner, is then moved into the furnace 2 into the position shown in the drawings, and the sliding doors 14 provided on the ends of the furnace are lowered to close the 90 openings in the ends of the furnace. The burners 3 are then ignited and the top surface of the furnace bottom 8 is thoroughly heated to the desired temperature after which the sintering operation is begun. A 95 stream of finely divided ore or other materials being sintered is then caused to flow through the opening 6 in the top of the furnace and, upon entering the furnace, being 100 deposited and spread over the furnace bottom in regulated quantities.

The sheet or stream of finely divided solids is brought into intimate contact with the highly heated products of combustion 105 within the furnace in falling from the opening in the furnace roof to the top surface of the furnace bottom. The materials are caused to become heated sufficiently to become soft or plastic so as to partly fuse and 110 stick together.

The materials as deposited upon the bot-

tom of the furnace within the furnace are spread over the surface of the furnace bottom by means of a rabble or other suitable tool, the tool being inserted in the openings provided for that purpose in the doors used in closing the ends of the furnace so as to distribute the materials in a layer of approximately even thickness over the furnace bottom.

10 By feeding regulated quantities of the materials in the furnace in a sheet or stream, a layer of sintered material of gradually increasing thickness is built up and agglomerated on the removable furnace bottom. After this mass has been built up to the desired height or thickness, the burners 3 are partly closed or are shut off. The furnace doors 14 are then opened and the furnace bottom 8 with the mass of partly fused or sintered material thereon is removed from the furnace. Another similar furnace bottom is then placed within the furnace, the bottom having been prepared in the meantime as described hereinbefore, and the above described sintering operation is then repeated, with a further supply of materials. The agglomerated materials, after being removed from the furnace, are allowed to cool until they are at the temperature best adapted to facilitate breakage into smaller lumps or pieces. The mass is then lifted from the framework of the furnace bottom and is broken up into pieces of the size desired for use in being charged 35 into a blast or other furnace, in which it is to be utilized, or other use for which the sintered material is intended. If care is taken during such cooling operations to break the material into lumps or pieces 40 while it is at a red heat and when the treated material does not have its greatest strength, very little difficulty will be had in breaking up the material into as small pieces as is necessary or desirable, and the labor 45 required and expense involved in breaking into pieces of the desired size will be lessened.

The advantages of my invention will be apparent to those skilled in the art. By introducing the materials gradually and in regulated quantities and causing the materials to pass through the zone of greatest heat within the furnace in falling from the roof to the furnace bottom, instead of heating a pile of the materials, the time required in agglomerating, or sintering a given quantity of the materials is greatly lessened, the expense connected therewith is reduced, and a body of semi-fused materials is quickly formed. By then subjecting the cooling mass to a series of blows at the time the mass has cooled sufficiently to lose its pasty or plastic condition and while it is still at a temperature approximating a red heat, the 60 so-formed mass is readily broken in pieces.

of suitable size for handling when found necessary or desirable.

Modifications in the construction and arrangement of the furnaces in which my improved method can be carried out will suggest themselves to those skilled in the art. A furnace having a removable top may be employed, a regenerative furnace can be used instead of the reverberatory furnace shown, and other changes may be made without departing from my invention as defined in the claims.

While the invention is primarily intended for use in sintering finely divided iron bearing materials such as ore, flue-dust, and mill scale, the invention is not to be restricted to any such use, but is intended to cover the sintering and agglomerating of finely divided solids generally within the scope of the appended claims.

I claim:

1. The method of sintering finely divided materials consisting in heating a layer of the material on the bottom of a sintering furnace to at least partly fuse the exposed surface thereof, directing a stream of fresh materials over the partly fused materials, and regulating the flow of the stream to permit the successive additions to become heated and thereby agglomerate with the materials on the furnace bottom, and removing the furnace bottom with the agglomerated materials thereon at intervals from the furnace.

2. The method of sintering finely divided materials consisting in spreading a layer of the material on the bottom of a sintering furnace, applying heat to at least partly fuse the exposed surface of the materials, adding fresh materials in a stream and spreading the additions over the partly fused materials on the furnace bottom, regulating the flow of the stream to permit the flowing stream to become heated as delivered into the furnace and thereby agglomerate with the material on the furnace bottom and removing the furnace bottom with the agglomerated materials thereon at intervals from the furnace.

3. The method of sintering finely divided materials consisting in heating and at least partly fusing a layer of the materials on the bottom of a sintering furnace, adding fresh materials in a stream, to the partly fused materials on the furnace bottom, regulating the flow of the stream of added material to permit heating thereof while passing through the furnace, removing the agglomerated furnace bottom and mass thereon from the furnace at intervals, and cooling and breaking the removed mass into pieces.

4. The method of sintering finely divided materials consisting in heating and at least partly fusing a layer of the materials on the bottom of a sintering furnace, directing a stream of fresh materials to flow into the

- furnace, regulating the flow of the stream to permit heating thereof while passing through the furnace and thereby agglomerate with the materials upon the furnace bottom, removing the furnace bottom with the agglomerated materials thereon at intervals from the furnace, cooling the removed mass and breaking the cooling mass into pieces.
- 10 5. The method of sintering finely divided materials consisting in spreading a layer of the materials on the removable bottom of a sintering furnace, placing the bottom in the furnace, heating and at least partly fusing the materials, adding a stream of fresh materials and spreading the additions over the furnace bottom, regulating the flow of the stream of added materials to permit partial fusion thereof while passing through the furnace and thereby agglomerate the materials on the furnace bottom, removing the bottom with the agglomerated materials thereon from the furnace at intervals, and removing the mass from the furnace bottom.
- 15 6. The method of sintering finely divided materials consisting in spreading a layer of the materials on the removable bottom of a sintering furnace, placing the bottom in the furnace, heating and at least partly fusing the materials, adding a stream of fresh materials and spreading the additions over the furnace bottom, regulating the flow of the stream of added materials to permit partial fusion thereof while passing through the furnace and thereby agglomerate with the materials on the furnace bottom with the agglomerated materials thereon, removing the bottom from the furnace at intervals, cooling the agglomerated mass and breaking the mass into pieces during the cooling operation.
- 20 7. The method of sintering finely divided materials consisting in spreading a layer of the materials on the removable bottom of a sintering furnace, placing the bottom in the furnace, heating and at least partly fusing the materials, adding a stream of fresh materials and spreading the additions over the furnace bottom, regulating the flow of the stream of added materials to permit partial fusion thereof while passing through the furnace and thereby agglomerate with the materials on the furnace bottom with the agglomerated materials thereon, removing the bottom from the furnace at intervals, cooling the agglomerated mass and breaking the mass into pieces.
- 25 8. The method of sintering finely divided materials consisting in spreading a layer of the materials on the removable bottom of a sintering furnace, placing the bottom in the furnace, heating and at least partly fusing the materials, adding a stream of fresh materials and spreading the additions over the

furnace bottom, regulating the flow of the stream of added materials to permit partial fusion thereof while passing through the furnace and thereby agglomerate with the materials on the furnace bottom, removing the bottom from the furnace at intervals, removing the mass from the furnace bottom, and breaking the mass into pieces.

9. The method of sintering finely divided materials consisting in spreading a layer of the materials on the removable bottom of a sintering furnace, placing the bottom in the furnace, heating and at least partly fusing the materials, adding a stream of fresh materials and spreading the additions over the furnace bottom, regulating the flow of the stream of added materials to permit partial fusion thereof while passing through the furnace and thereby agglomerate with the materials on the furnace bottom with the agglomerated materials thereon, removing the bottom from the furnace at intervals, cooling the agglomerated mass and breaking the mass into pieces.

In testimony whereof, I have hereunto set my hand.

JAMES G. WEST, JR.

Witnesses:

EDMUND D. NUGENT,  
CHAS. J. SCHUCK.